

Nov. 1, 1966

V. E. CULLER

3,283,155

SHORT-DURATION LIGHT SOURCE COMPRISING AN ELECTRON  
IRRADIATED TRANSPARENT INSULATING BODY  
Filed June 5, 1963



**FIG. 1**



**FIG. 2**

INVENTOR  
Vaughn E. Culler

BY Clarence R. Patty, Jr.  
ATTORNEY

## 1

3,283,155

SHORT-DURATION LIGHT SOURCE COMPRISING  
AN ELECTRON IRRADIATED TRANSPARENT  
INSULATING BODYVaughn E. Cuiller, Pennington, N.J., assignor to Corning  
Glass Works, Corning, N.Y., a corporation of New  
York

Filed June 5, 1963, Ser. No. 285,792

3 Claims. (Cl. 250—84)

The present invention relates to sources for producing light pulses of very short duration and to methods for producing such sources.

An object of the invention is to provide a source of light pulses having durations of the order of one microsecond.

A further object is to provide such a light source which is capable of storing for long periods the electrical charge necessary to produce such a light pulse.

Another object is to provide a simple and inexpensive flash source for use in photography.

These and other objects, which will be apparent from the description, are accomplished by irradiating a transparent insulating material having certain electrical characteristics in order to provide a localized excess of electrical charge in one portion of the material and subsequently disrupting the charge distribution to effect an electrical discharge which produces a light pulse.

The invention will be described with reference to the accompanying drawing, in which:

FIGURE 1 illustrates the process whereby a light source according to the present invention is produced, and

FIGURE 2 illustrates a light source in condition to be discharged to produce a light pulse.

It has previously been known that it is possible to collect electrical charges in insulating materials and that subsequent discharge, either spontaneous or intentional, may produce lightning-like flashes of light. Until the present time, however, it has not been possible to store such charges for times sufficient to permit the use of such materials as light sources for commercial application, such as photography, and for this reason such materials have been of academic interest only. Accordingly, the present invention involves both the recognition that transparent insulating materials having localized electrical charges may be used as light sources for photographic application and that such materials, when chosen to have particular electrical characteristics, may store such charges for times sufficient for commercial photographic use.

It is known that charged insulators lose their charge according to the equation:

$$q = q_0 \exp(-t/T) \quad (1)$$

where  $q$  is the charge density at time  $t$ ,  $q_0$  is the charge density at time 0, and  $T$  is a time constant characteristic of the insulator. The same time dependence is also known to be true for the internal electric field in an insulator.

The time constant can be derived as

$$T = 8.85 \times 10^{-14} K \rho \quad (2)$$

where  $T$  is in seconds,  $K$  is the relative dielectric constant and  $\rho$  is the resistivity of the insulator in ohm-cm.

It is known that a material will absorb only a limited amount of electrical charge at a localized portion of the material before electrical breakdown. In order for such material to be usable as a practical commercial light source, it is necessary for such charge, or a substantial part thereof, to be retained for some length of time. In the case of glasses and plastics, it has been found that for practical use, the material must retain on the order of 37% of the original deposited charge in order for it

## 2

to be useful as a photographic light source. From Equation 1, it can be determined that when the time  $t$  is equal to the time constant  $T$ , both the electrical charge and the electrical field decay to about 37% of their original values. Initially it was assumed that for a charged glass or plastic material to have utility as a light source, a useful life of 90 days is required. Thus, the charge and field may decay to 37% of their original value in a period equal to 90 days, and will do so when the time constant  $T$  equals 90 days.

In order to calculate a preliminary value for the product  $K \rho$ , the required value of the time constant  $T$  was substituted in Equation 2, and a tentative value of the product  $K \rho$  for adequate electric charge retention was determined as approximately  $10^{20}$  ohm-cm.

There is evidence that at very high electric field strengths resistivity does not have the same value that it has at lower field strengths. In addition, it is difficult to determine the correct dielectric constant except with nearly ideal insulators. For these reasons, the calculated required value of  $K \rho$  was verified empirically by irradiating various glass samples having values of  $K \rho$  centering around  $10^{20}$  ohm-cm. The experimental results indicate that although most materials having  $K \rho$  equal to or greater than  $10^{20}$  ohm-cm. exhibit adequate charge retention, a preferred value of at least  $10^{22}$  ohm-cm. is necessary in order to insure a life of 90 days in all materials.

Additional experimentation has shown that certain glasses, for example vitreous silica, exhibit large increases in electrical conductivity during irradiation. Such glasses, even though exhibiting the required  $K \rho$  under normal conditions, cannot be charged sufficiently for use as light sources. It has been found that in order for a localized charge of sufficient magnitude to be built up, it is necessary that  $K \rho$  be greater than  $3 \times 10^{16}$  ohm-cm. during irradiation.

Although the present invention is not to be limited thereby, the following is given as a preferred embodiment of the invention:

Blocks of glass, such as 10, in the shape of right circular cylinders two inches in diameter and one-fourth inch thick were ground and polished. The glass had a composition 58%  $\text{SiO}_2$ , 15%  $\text{Al}_2\text{O}_3$ , 9%  $\text{CaO}$ , 8%  $\text{MgO}$ , 6%  $\text{BaO}$  and 4%  $\text{B}_2\text{O}_3$ . The extrapolated room temperature resistivity of the glass was  $10^{24}$  ohm-cm., and its dielectric constant was about 6.4.

One flat side of each block was exposed to 2 mev. electron irradiation. The total exposure was 1.2 megarads, and was attained at 0.1 megarad per pass through the electron beam. After exposure the blocks were stored for periods up to six months. Each block, when removed from storage and struck with a metal rod, emitted a bright flash of light having a duration which was measured to be about one microsecond.

When a single irradiated block was discharged  $15\frac{1}{2}$  inches from a 12 inch diameter disc rotating at 3650 revolutions per minute and having thereon radial lines separated by 0.45 mm., a photograph taken at a camera setting of  $f/2$  with a film having a speed rating of 800 ASA clearly resolved the radial lines.

Glass blocks irradiated according to the present invention exhibit over conventional high-speed flash sources the advantages of compact size and low cost.

Light sources according to the present invention may be produced utilizing any transparent material having the described electrical characteristics. Localized concentrations of electrical charges may be produced by irradiation with electrons, as in the described embodiment, by irradiation with gamma rays, which cause electrons in the material to move away from the radiation source, or by irradiation with protons.

The light emitted from electron-irradiated glass blocks is essentially white light and can be used for taking satisfactory color photographs. It is of interest that, although such irradiated glass blocks pick up positive charges from the atmosphere and are accordingly electrically neutral, if such blocks have the above-described electrical characteristics, the localized electrical fields necessary for the production of light pulses remain.

When blocks larger than those described above are utilized, both the magnitude and the duration of the resultant light pulse are increased, and blocks of varying shapes may be used, as dictated by considerations such as reflector shape when such blocks are utilized in photography.

It is to be understood that although the above-described limitations on the value of the quantity  $K_\rho$  are necessary if light sources according to the present invention are to be used for conventional photographic applications, there will be some instances in which substantial storage times are not required, and in such instances the normal value of the quantity  $K_\rho$  may be less than  $10^{20}$  ohm-cm. In all cases, however, regardless of the required storage time, the value of  $K_\rho$  during irradiation must be at least equal to  $3 \times 10^{16}$  ohm-cm.

It will be understood that the foregoing has been given merely as a description of a preferred embodiment of the present invention. Accordingly, it is intended that the invention be limited only by the scope of the appended claims.

What is claimed is:

1. A light source comprising a transparent material having the normal product of its electrical resistivity and its dielectric constant equal to at least  $10^{20}$  ohm-cm. and

having during electron irradiation the product of its electrical resistivity and dielectric constant equal to at least  $3 \times 10^{16}$  ohm-cm., said material having concentrated in a portion thereof an excess of negative electrical charges.

5 2. A light source comprising a glass body having the normal product of its electrical resistivity and its dielectric constant equal to at least  $10^{22}$  ohm-cm. and having under electron irradiation the product of its electrical resistivity and its dielectric constant equal to at least  $3 \times 10^{16}$  ohm-cm., said body having concentrated in a portion thereof an excess of negative electrical charges.

10 3. The method for producing a light source which comprises irradiation with electrons one part of a transparent insulating body normally having the product of its electrical resistivity and its dielectric constant equal to at least  $10^{20}$  ohm-cm. and having during irradiation the product of its electrical resistivity and its dielectric constant equal to at least  $3 \times 10^{16}$  ohm-cm. in order to build up in said part of said body an excess of negative electrical charge.

#### References Cited by the Examiner

#### UNITED STATES PATENTS

|    |           |        |                  |       |        |
|----|-----------|--------|------------------|-------|--------|
| 25 | 2,990,473 | 6/1961 | Kallmann         | ----- | 250—71 |
|    | 3,093,735 | 6/1963 | Blakewood et al. | ----- | 250—83 |
|    | 3,165,631 | 1/1965 | Solow et al.     | ----- | 250—42 |

RALPH G. NILSON, *Primary Examiner.*

30 H. S. MILLER, A. R. BORCHELT, G. E. MATTHEWS,  
*Assistant Examiners.*